

June 13, 1933.

A. LEFERE

1,913,492

## METHOD OF WHEEL HUB FORGING

Filed Aug. 3, 1931

2 Sheets-Sheet 1

Fig 1.



Fig. 2.



June 13, 1933.

A. LEFERE

1,913,492

METHOD OF WHEEL HUB FORGING

Filed Aug. 3, 1931

2 Sheets-Sheet 2

*Fig. 3.*



*Fig. 4.*



INVENTOR.

ALIDOR LEFERE  
BY Barnes & Tisselle  
ATTORNEYS.

## UNITED STATES PATENT OFFICE

ALIDOR LEFÈRE, OF JACKSON, MICHIGAN, ASSIGNOR TO LEFÈRE FORGE & MACHINE COMPANY, OF JACKSON, MICHIGAN, A CORPORATION OF MICHIGAN

## METHOD OF WHEEL HUB FORGING

Application filed August 3, 1931. Serial No. 554,658.

This invention relates to a new automobile wheel hub together with a novel method of forming the same.

Most wheel hubs are formed by a metal stamping operation out of sheet metal, or are made in the form of malleable steel castings, or else are formed from metal forgings which have to be drilled and machined to get the proper dimensions and shape.

10 It has been proposed to forge car wheels and their hubs by forging die operations and coincident piercing or punching operations. So far as I am aware no satisfactory method has been proposed or utilized for forging 15 automobile wheel hubs and shaping them to substantially the final form in a forging operation.

I accomplish this object by so designing the final forging blank and the final forging 20 product as to provide a suitable relief for the extruded metal in punching the slug out and expanding the shell to give it the final shape. This relief is not only useful in accommodating 25 the flow of the metal and preventing the freezing or binding of the punch and dies but also permits of the handling of slightly varying blanks due to varying heats.

Referring to the drawings:

Fig. 1 is a vertical section through the dies 30 before they are brought together.

Fig. 2 is a similar view when they first come into contact.

Fig. 3 is a similar view of the dies at or near the finish of their downward movement.

35 Fig. 4 shows the dies separated and the slug ejected.

Numeral 1 designates the base of the forging machine having a bed 3 which carries a trimming die 2 which is arranged to shear off or trim the flash 4 on the blank when the upper and lower dies are driven down. The sleeve 5 is upwardly pressed by a heavy helical spring 6. At the top of the sleeve rests a lower forming die 7 having an upper face 40 arranged to give the final shape to the inside face of the hub flange. The upper die 8 has its lower face arranged to finally shape the outside face of the hub flange while the center of the die is arranged to form the outside 45 surface of the body of the hub. This occurs

when the metal is arranged to flow by means of the punch 9 which also forms a mandrel with which the upper die cooperates.

Referring now to Fig. 1: This shows the hub blank after it is taken from the forging hammer and placed in the final forging dies. The blank has been formed in the customary way of forming forgings from hot billets or sections of metal. The blank has been pounded into a general approximation of the 60 contour the hub is finally to have. A pad 11 has been left between the upper and lower die at the center. It will also be noticed that a peripheral relief 12 encircles the outer end of the body of the hub. This relief is 65 considerably reduced in Figs. 3 and 4 at the point 12a by the flow of the metal to give the final forging dimensions at the outer end of the hub and to make the inside and outside surfaces substantially cylindrical. 70 In achieving this the blank at the outer end is tapered and made considerably smaller in diameter than the final product. The stationary punch 9 is carried on the upper end of the stationary post 14. The upper die 8 75 which may be operated by any suitable ram and press mechanism (not shown) comes down onto the work and the lower die leaving the ejector rod 15 suspended above. This is shown in Fig. 2. This shears off the 80 flash as already referred to. The work is then driven over the end of the stationary punch 9 and this acts also in connection with the upper die to punch out the slug 16 and cause the material to flow out against the 85 center opening of the upper die and fill up part of the relief as shown in Fig. 3 at the same time the ejector rod 15 comes down. The slug 16 cools less rapidly than the end 90 of the hub and consequently will not drop back into the end of the hub as the lower die rises with the spring pressure. If the slug sticks in the upper die then it is promptly ejected by the ejector rod 15 as shown in 95 Fig. 4.

The large relief space on the outside of the body of the hub affords a space into which the metal can flow as the pad is punched out. By reason of a liberal excess of relief 100 no difficulty is experienced in handling

blanks of a slightly varying size due to the varying heats or forging operations. By relieving this flow of the metal any difficulty in the binding of the dies or the punch is avoided. The excess relief results in what I call a residual groove 12a. Furthermore, the relief forms a space into which the punch or mandrel can cause the metal to flow to form a substantially accurate outside and inside diameter at the end of the hub.

This method of forging and finishing the hub eliminates some of the machine operations such as boring, etc. which have been thought necessary in manufacturing of forged wheel hubs. These machine operations increase both the labor and material costs.

The operations which have just been described may or may not be carried out in the same heat with which the blank is formed from the billet or bar.

What I claim is:

1. The method of manufacturing wheel hubs which comprises the forging of a blank having a hub flange and a hollow hub body except for a pad to keep the dies separated, the body being provided with a relief on its periphery of excess capacity, subjecting said blank while in heated condition to a final forging by punch and die operation in which the pad is punched out and the body at one end is expanded and the metal of the body caused to flow by reason of the excess relief and to establish substantially the dimensions and shape desired for the final product and leave a peripheral groove resulting from the said relief.

2. The method of manufacturing wheel hubs which comprises the forging from a hot billet of a blank with a suitable flange and body portion in which the body portion is on the exterior given a substantial relief with the body hollow except for a pad, then subjecting the blank while in the heated condition to a final forging by punch and die operation in which the pad is punched out the end of the body expanded and by reason of the relief the metal is caused to flow coincident with the punching to permit the punching and shaping the hub body into substantially the final dimensions and contour desired, while leaving a residual space resulting from the relief space, the punch being drawn back out of the work.

3. The method of manufacturing wheel hubs which comprises the forging of a blank with flange and hollow body except for a transverse pad, said body having an external relief space of excess capacity at its outer end, and then the placing of the forging blank between two dies which encompass the outside of the body and the hub flange and then moving the dies relatively to a punch which forces out a slug of metal in eliminating the pad and expands the outer end of the

body into one of the dies and the relief space to properly shape the exterior and the interior circumference, while leaving a residual space resulting from the relief space punch being drawn back out of the work.

In testimony whereof I affix my signature

ALIDOR LEFER